# EUROPEAN PATENT APPLICATION

(11) **EP 4 144 446 A1**
(43) Date of publication of application: **08.03.2023**
(21) Application number: 21195406.0
(22) Date of filing: 07.09.2021
(51) Int. Cl.: B05D 3/10, B05D 3/12, B05D 5/08, B05D 7/14, B05D 7/00, B05D 1/40

(54) **POLYMER COATED SHEET PRODUCT AND METHOD OF MANUFACTURING IT**

(71) Applicant: TATA STEEL UK Limited, London SW1P 4WY (GB)
(72) Inventor: Barker, Peter, 1970 CA IJmuiden (NL); Johnson-Oughtibridge, Emily, 1970 CA IJmuiden (NL); Stevens, Natasha Kate, 1970 CA IJmuiden (NL)
(74) Representative: Wynne-Jones IP Limited

(57) **Abstract**

Polymer coated sheet product comprising a metallic substrate provided with a polymer coating, the polymer coating comprising an inner polymer layer contacting the metallic substrate and an outer polymer layer wherein an emboss pattern is hot embossed in the outer polymer layer.

## Description

The invention relates to a polymer coated sheet product and a method of manufacturing it. In particular it relates to a polymer coated sheet that has an emboss.

Such an embossed polymer coated sheet is known e.g. in the form of organic coil coated steel sheet coated with a PVC layer having an emboss.

In the known organic coated product the PVC layer has a thickness of around 200 microns, with an emboss of between 50 and 70 microns.

The known product has several disadvantages: One is that it contains PVC which is considered to have inferior sustainability credentials. Another is that it uses in the order of 200 microns of polymer coating. Still another is that it has a low fire resistance classification, and finally it has perceived weaknesses in strong UV and hot climates.

The objective of the invention is to provide an improved polymer coated sheet product that has an emboss.

Another objective of the invention is to provide a non-PVC-containing product that is not based on PVC polymer technology.

Another objective is to provide a product that is environmentally friendly and can be manufactured in a more cost effective way.

Still another objective is to produce a polymer coated sheet product that has a combination of excellent corrosion resistance and UV resistance together with a unique emboss to provide a mark of authenticity

In order to realise one or more of the objectives according to the invention the polymer coated sheet product is provided that comprises a metallic substrate provided with a polymer coating, the polymer coating comprising an inner polymer layer contacting the metallic substrate and an outer polymer layer wherein an emboss pattern is hot embossed in the outer polymer layer which is of PVDF. By having the outer polymer layer of PVDF an improved polymer layer structure is realised, having a considerably smaller thickness than the known polymer coated embossed sheet product.

In an embodiment there is an intermediate polymer layer extending between the inner polymer layer and the outer polymer layer. This achieves an improved product performance compared to a two polymer layer product that matches or surpasses the known PVC product performance. The intermediate layer may provide the required colour with excellent colour stability and also is receptive to the outer layer and embossing.

In an embodiment the inner polymer layer is of polyester, polyurethane or acrylic. Such an inner layer provides both excellent corrosion resistance and the required long term adhesion between the pretreatment and subsequent polymer layers.

In an embodiment the intermediate polymer layer is of polyester, polyurethane or PVDF resin. This achieves the effect that the intermediate polymer layer chemistry provides a long term colour performance but also improved fire resistance properties.

In an embodiment the dry film thickness of the whole polymer coating is more than 20 microns. This achieves the effect that the polymer coating provides the required barrier properties regarding corrosion and colour fastness.

In an embodiment the dry film thickness of the whole polymer coating is less than 100 microns. This achieves the effect that the optimum product thickness is reached to ensure the required performance properties but also sustainability by using less raw materials than the current product.

In an embodiment the inner polymer layer has a dry film thickness of 3-30 microns, preferably 5-25 microns.

In an embodiment the outer polymer layer has a dry film thickness of 20-70 microns, preferably 30-50 microns. Hereby the required emboss depth and clarity is achieved through the outer polymer layer whilst still maintaining the required barrier performance of the outer coating.

In an embodiment comprising an intermediate polymer layer extending between the inner and the outer polymer layer the intermediate polymer has a dry film thickness of 10-25 microns. Hereby the required colour fastness and opacity is achieved and/or the product performance requirements are met with the greatest possible colour range for the most cost-effective amount of coating.

In an embodiment wherein there is an intermediate polymer the total dry film thickness of the intermediate polymer and the outer polymer layers is at least 20 microns. Hereby the required emboss depth and clarity is achieved through the outer polymer whilst still maintaining the required barrier performance of the intermediate and outer polymer layer.

In an embodiment the metallic substrate comprises a steel sheet. The steel sheet provides the structural integrity for further processing the product into components for the construction industry.

In an embodiment the steel sheet has a metallic coating, such as of Zn or a Zn alloy, or a Zn-Mg-Al alloy or of any other metal or alloy. The metallic coating provides a combination of barrier and sacrificial protection for the underlying steel substrate.

In an embodiment the metallic substrate comprises an aluminium sheet. The aluminium sheet provides a corrosion resistant substrate.

The invention is also embodied in a method of manufacturing a polymer coated sheet product having an emboss comprising the following consecutive steps:
- providing a metallic substrate such as S220GD to S550GD or DX51 to DX56 in a suitable gauge ranging from 0.2 to 1.5 mm;
- applying as a first polymer layer an organic primer with a dry film thickness of between 3 and 30 microns, the primer being either polyester or polyurethane or acrylic based and curing the primer;
- optionally applying one or more further polymer layers, the or each further polymer layer being either a colour polymer layer or a base colour polymer layer, having a polyurethane or PVDF chemistry and curing, each colour or base colour polymer layer being preferably between 10 and 30 microns and to be cured preferably between 230 °C and 250 °C;
- applying a final polymer layer being either a clear or a colour PVDF polymer layer with a minimum dry film thickness of 20 microns and a maximum dry film thickness of 70 microns;
- curing the final polymer layer in a curing station preferably at a peak metal temperature of 240 °C to 250 °C;
- embossing the still hot product by passing it through an embosser station as soon as the product exits the curing station whereupon while the product is still hot, a desired pattern is embossed directly into the PVDF final polymer layer, the emboss pattern depth on the embossing roll being preferably 20 microns to 70 microns;
- quenching the final polymer layer by passing the product through a quenching section to cool it whereby the emboss is fixed within the final polymer layer.

According to this method the outer layer that comprises the embossing is of PVDF which achieves the effect that the thermoplastic nature of the specially designed polymer formulation receives an emboss from the hot embossing process.

Especially if the coating and embossing takes place in one coating line and the applying of all the polymer layers and the hot embossing take place in one pass through the manufacturing line, this process is a very cost effective way of manufacturing the product.

In an embodiment the metal substrate is coated with a metallic coating on the metal substrate.

In an embodiment the metallic coating is a zinc based coating like a Zn coating, a Galvalloy coating, a Galvalume coating, or a Zn-Mg-Al coating, with a coating weight of 60 to 600 grams per square metre. This achieves the effect that the metallic coating weight enables both barrier and sacrificial protection of the steel substrate.

In an embodiment the optionally metallic coated substrate before applying the primer is cleaned involving an alkali cleaning process to remove residual organic matter and metallic oxides. The alkali cleaning process removes the residual contaminants and oxides present on the metallic coated surface.

In an embodiment the optionally metallic coated substrate before applying the primer is pretreated by passing it through a chromate free pretreatment bath based on titanium dioxide or an inorganic component together with an organic polymer to improve the corrosion resistance and enable optimal adhesion between the metallic substrate and subsequent organic polymer layers. The titanium based pretreatment is applied to provide the required corrosion resistance and adhesion between the inorganic metallic coating and subsequent polymer layers.

In an embodiment the pretreated substrate is rinsed and dried in an oven. This achieves the effect that all residual pretreatment solution is removed prior to the next application process.

Further benefits and advantages of the present invention will become apparent after a careful reading of the description of investigations and examples with appropriate reference to the accompanying drawings.

In the drawings:
Fig. 1 is a photograph of the 50 micron emboss roll with scintilla pattern.
Fig. 2 is a selection of microscope images showing samples with different emboss quality, it shows in A an excellent emboss, in B a faint/poor emboss, in C a faint/poor emboss and in D an unembossed sample.
Fig. 3a is showing the surface profile map of a sample with good emboss produced with the 50 micron emboss roll at a set pressure of 6.5 bar. This pressure is the pressure that is read on a meter and that can be calculated into a force which is indicated in table 1.
Fig. 3b is showing the surface profile map of a sample with a poor emboss produced with the 50 micron emboss roll at a set pressure of 4.5 bar.
Fig. 4 is a graph showing the contact angles of PVDF outer layer coatings on different coated substrates. On the horizontal axis, 1 concerns a PUR primer formulation, 2 concerns a polyester primer formulation, 3 concerns a PUR formulation that could be used for the intermediate polymer layer, and 4 concerns a colour PVDF formulation that could be used for the intermediate or the outer polymer layer and on the vertical axis the contact angles of the respective formulations are shown in degrees.

Although the invention has been explained in relation to its preferred embodiment(s) as mentioned above, it is to be understood that other possible modifications and variations can be made without departing from the scope of the present invention. It is, therefore, contemplated that the appended claim or claims will cover such modifications and variations that fall within the true scope of the invention.

### Examples

Hereinafter, the present invention is described in more detail and specifically with reference to the examples, which however are not intended to limit the present invention.

### Example 1

Line produced pretreated and primed samples of Galvalloy were used for the embossing experiments. A 0.675 mm gauge Galvalloy substrate was precleaned, a Cr-free pretreatment based on Titanium was applied and subsequently thereon a nominal 25 microns Cr-free polyurethane primer was applied using a polymer coil coating line. This primer only material was cut into 310 x 210 mm size samples for investigation.

In the course of the investigation, various colour layers of either a polyurethane (nominal 25 microns) or PVDF chemistry (nominal 20 microns) were applied via bar coating over the primer only material. Via the use of a calibrated thermocouple, the peak metal temperature (PMT) was accurately determined during curing in an oven. The cured panels were subsequently quenched to room temperature, dried before the final polymer layer was applied.

The final polymer layer was a clear PVDF chemistry which for the purposes of this study was applied at a thickness between 20 and 48 microns before curing at a PMT of 249 °C. Via the use of a calibrated thermocouple, the peak metal temperature (PMT) was accurately determined during curing in an oven. After the panels had cured, the panels automatically exited the oven and the panels were either directly transferred to the embossing unit or left on a tray to cool down to a lower temperature as measured by the thermocouple (embossing temperature) before placing the coated panel into the embossing unit.

At the desired embossing temperature, the sample was fed into the embossing unit having a motor driven backing rubber roll with diameter 10.5 cm and a top embosser roll with diameter 7 cm that is not driven. As the sample entered the embossing unit the temperature was recorded after which the thermocouple was removed just before the sample entered the embossing roll so as to not damage the equipment. By means of a pneumatic actuator the top embosser roll was pressed onto the backing rubber roll with an applied force F in N as indicated in table 1 below.

The embosser roll depth is defined as the difference between the maximum and minimum radius of the emboss roll was 50 microns. After embossing the embossed sample was immediately quenched in cold water.

The embossed samples were then visually assessed for the result and quality of the emboss and any defects. The quality and topography of individual emboss logos were quantified by surface profile analysis and Scanning Electron Microscopy (SEM).

Table 1 shows the results and quality of emboss for variants of intermediate polymer layer thickness and chemistry, outer polymer layer thickness and chemistry, embossing temperature and embossing pressure. The laboratory work clearly substantiates the invention in confirming the optimum polymer chemistries, emboss temperature and emboss pressure to achieve the required emboss pattern in the outer polymer layer.

**Table 1**

| No. | intermediate layer chemistry | outer layer thickness | emboss temperature | emboss pressure in bar | applied force N | result and quality |
|---|---|---|---|---|---|---|
| 1 | PUR 25µm | PVDF 20µm | 249 °C | 4.5 | 118.17 | unembossed |
| 2 | PUR 25µm | PVDF 20µm | 249 °C | 6.5 | 170.57 | unembossed |
| 3 | PUR 25 µm | PVDF (p) 20µm | 249 °C | 4.5 | 118.17 | unembossed |
| 4 | PUR 25 µm | PVDF (p) 20µm | 249 °C | 6.5 | 170.57 | unembossed |
| 5 | PUR 25µm | PVDF 30µm | 249 °C | 4.5 | 118.17 | unembossed |
| 6 | PUR 25µm | PVDF 30µm | 249 °C | 6.5 | 170.57 | poor emboss |
| 7 | PUR 25µm | PVDF (p) 30µm | 249 °C | 6.5 | 170.57 | poor emboss |
| 8 | PUR 25µm | PVDF 40µm | 249 °C | 4.5 | 118.17 | poor emboss |
| 9 | PUR 25µm | PVDF 40µm | 249 °C | 6.5 | 170.57 | excellent emboss |
| 10 | PUR 25µm | PVDF (p) 40µm | 249 °C | 6.5 | 170.57 | excellent emboss |
| 11 | None | PVDF (p) 40µm | 249 °C | 6.5 | 170.57 | excellent emboss |
| 12 | None | PVDF 40µm | 249 °C | 6.5 | 170.57 | excellent emboss |
| 13 | PUR 25µm | PVDF 40µm | 234 °C | 6.5 | 170.57 | excellent emboss |
| 14 | PUR 25µm | PVDF 40µm | 219 °C | 6.5 | 170.57 | poor emboss |
| 15 | PVDF 20µm | PVDF 30µm | 249 °C | 6.5 | 170.57 | over-embossed |
| 16 | PVDF 20µm | PVDF 40µm | 249 °C | 6.5 | 170.57 | over-embossed |
| 17 | PVDF 20µm | PVDF (p) 40µm | 249 °C | 6.5 | 170.57 | over-embossed |
| 18 | PUR 25µm | PUR 30µm | 249 °C | 6.5 | 170.57 | unembossed |
| 19 | PUR 25µm | PUR 40µm | 249 °C | 6.5 | 170.57 | unembossed |
| 20 | PUR 25µm | FEVE 30µm | 249 °C | 6.5 | 170.57 | unembossed |
| 21 | PUR 25µm | FEVE 40µm | 249 °C | 6.5 | 170.57 | unembossed |
| 22 | PUR 25µm | PVDF 48 mu | 249 °C | 4.5 | 118.17 | Poor emboss |
| 23 | PUR 25µm | PVDF 48 mu | 249 °C | 6.5 | 170.57 | Good emboss |

| | | | | | | |
|---|---|---|---|---|---|---|
| PVDF = Polyvinylidene difluoride, clear unless stated (p)=pigmented PUR = Polyurethane, pigmented FEVE = Fluoroethylene vinyl ether, clear | | | | | | |

For the microscopy evaluation of the emboss quality reference is made to Fig. 1 representing excellent emboss, poor emboss and unembossed.

In carrying out the experiments, it occurred to the inventors that the first thing to get right is the thickness of the "embossable layer". If it is PVDF in the intermediate polymer layer and in the outer polymer layer you could sum the layers and call that the embossable layer. But if you have PUR as the intermediate polymer layer and PVDF as the outer polymer layer you would have to increase the thickness of the PVDF outer polymer layer to a minimum suitable for embossing.

Using SEM cross sections of the samples the quality of the embossed product was assessed. In a good sample the low point of the outer polymer layer was approximately 35 microns, and the high point of the outer polymer layer was approximately 75 microns. Over embossing should be avoided as this can have detrimental effects on long term product performance. SEM can help to show the overall integrity of the embossed coating system.

### Example 2

Galvalloy samples that were line produced, pretreated and provided with a primer as described in Example 1 were used in Example 2. Also in this example the emboss roll depth was 50 microns.

In this investigation, the intermediate and outer layer polymer chemistry composition was investigated to determine the optimum combination for embossing. Based on Example 1, the following parameters were kept constant during the investigation; embosser roll depth of 50 microns, outer polymer layer thickness of 40 microns, outer layer polymer chemistry to be a composition of PVDF, embossing temperature of 249 °C and embossing pressure of 6.5 bar.

Table 2 shows the results and quality of emboss for the variants of the intermediate and outer layer chemistry composition.

**Table 2**

| No. | intermediate layer (pigmented) | outer layer | comments |
|---|---|---|---|
| 24 | PUR 25µm with polyamide beads | PVDF 40 µm clear, soft resin | emboss fair |
| 25 | PUR 25µm with no polyamide beads | PVDF 40 µm clear, soft resin | emboss excellent |
| 26 | PVDF 20µm | PVDF 40 µm clear, soft resin | over-embossed |

| | | | |
|---|---|---|---|
| PVDF = Polyvinylidene difluoride, clear or pigmented PUR = Polyurethane, clear or pigmented PES = Polyester | | | |

The key to embossing is the flow of material between the substrate and the emboss roll during the emboss process. In a roll to roll coating process between two flat rolls the successful formation of the film is dependent on the flow of the coating through the roll nip. Hot embossing still has a need for flow of the material to be embossed. Thermoset polymers such as PU or FEVE tested in this study cannot flow once cured. Thermoplastics have a range around their glass transition temperature (Tg) in which the material can flow. As the emboss roll impresses a pattern into the surface the polymer material must flow well enough in the space available to form the shape required and then hold that shape on exit long enough for the embossed film to be quenched setting the emboss pattern.

The wettability is an indication of how well a material will flow over the surface during both the film formation and the emboss step.

The formulation wettability on different surfaces was examined as follows. The flow of the coating formulation during the embossing process is key to the final emboss quality and to compare this behaviour in complete coating systems a droplet of the respective formulation was allowed to spread on different underlying polymer layers. These results show the importance of the underlaying surface in determining the flow behaviour of embossed layers in the production process. The more wettable the thermoplastic polymer mix, the higher the flow rate. The three tested coatings were all PVDF formulations. They showed greater wettability on PVDF intermediate layer surfaces compared to PUR intermediate layers and a greater wettability of PES primers compared to PUR primers.

As is shown in figure 4, it turns out that it is a critical factor for embossibility to have a contact angle on any surfaces of at least 12.

Static contact angle measurements were completed by placing a droplet of a polymer (1 cm³) onto a substrate and measuring the contact angle with a pocket goniometer (model PGX) and PG software. An average of at least three readings were taken for each variable.

### Example 3a

The interaction between the embossed layer and the underlying surface (intermediate layer or primer) on emboss quality was studied. Samples were embossed at 6.5 bar with a 50 micron emboss roll after curing at 249 °C. The results support the finding that an increased wettability of the outer layer improves the final emboss quality.

**Table 3**

| No. | primer | Intermediate layer | PVDF, contact angle as measured | emboss quality at 20 microns PVDF | emboss quality at 40 microns PVDF |
|---|---|---|---|---|---|
| 27 | PUR 25µm | None | 36.2 | poor | good |
| | | | 20.4 | good | excellent |
| | | | 31.0 | poor | good |
| 28 | PES 10µm | None | 18.2 | poor | good |
| | | | 12.6 | good | excellent |
| | | | 14.5 | poor | good |
| 29 | PUR 25µm | PUR 25µm | 44.4 | unembossed | good |
| | | | 35.9 | poor | excellent |
| | | | 40.0 | poor | good |
| 30 | PES 10µm | PVDF 20 µm | 14.4 | excellent | excellent |
| | | | 12.8 | excellent | excellent |
| | | | 19.9 | good | excellent |
| 31 | PES 10µm | PUR 25µm | 44.4 | unembossed | good |
| | | | 35.9 | poor | excellent |
| | | | 40.0 | poor | good |

### Example 3b

The dependency of emboss quality on the combination of film thickness and layer chemistries was studied. All samples were produced with a 50µm embosser roll at 6.5 bar and at a PMT of 249 °C for the outer polymer layer. The results show that the final emboss quality is determined by both the formulation and thickness of individual layers in the overall composition of the coating system.

### Example 4

Samples have been produced using different pattern depth emboss rolls. The 30 micron roll has a smaller gap to fill than the standard 50 micron, 70 micron roll has a larger gap. This affects the flow of material. For the 30 micron too high a thickness of embossable coating decreases the flow of material so as to decrease the quality of emboss. Table 4 shows the results of a PVDF layer embossed with 30 micron emboss roll at 6.5 bar cured at 249 °C.

**Table 4**

| primer | Intermediate layer | outer layer PVDF | emboss Quality |
|---|---|---|---|
| PUR | none | 20 microns | Poor |
| PUR | PUR 25microns | 20 microns | unembossed |
| PES | None | 20 microns | poor |
| PES | PVDF 20 microns | 20 microns | poor |
| PUR | none | 40 microns | poor |
| PUR | PUR 25 microns | 40 microns | unembossed |
| PES | None | 40 microns | Poor |
| PES | PVDF 20 microns | 40 microns | Poor |

Over-embossing was seen in samples embossed with a 70 micron emboss roll at 6.5 bar pressure cured at 249 °C. This occurs when the size of the emboss pattern does not restrict flow in the outer polymer layer but there is not enough material to form the emboss pattern in the outer polymer layer. This causes the pattern to cut through the underlying coating system compromising performance. Table 5 shows examples for a 70 microns emboss roll at 6.5 bar cured at 249 °C.

**Table 5**

| primer | intermediate layer | outer layer | comments |
|---|---|---|---|
| PUR 25µm | PUR 25 µm | PVDF 40 µm | Good Emboss |
| PES 10 µm | PVDF 20 µm | PVDF 40 µm | Over embossed |
| PES 10 | none | PVDF 40 | over embossed |
| PUR 25 | none | PVDF 40 | over embossed |

It is remarked that the line speed may influence the quality of an emboss on a coating film. The higher the line speed the less time the pattern is held on the surface of the coating and so the faster the polymer will need to flow to fill this gap. The line speed of a continuous coating line is normally determined by the required speed to achieve the cure through the ovens. Experiments at different roll speeds show that improvements of the quality of the emboss can be seen at higher speeds.

### Example 5

Changing the emboss pattern can influence the final quality of the embossed coating. A more intricate pattern of a similar depth will emboss less effectively than that of a less intricate pattern.

Emboss rolls with two different patterns were used - the standard scintilla as used in previous examples and an overlapping T design. Both had emboss pattern depths of 50 microns +/-5 microns.

**Table 6**

| emboss pattern | emboss layer thickness | emboss quality |
|---|---|---|
| scintilla | 20 microns | okay/poor |
| overlapping T (more intricate) | 20 microns | no emboss |
| Scintilla | 40 microns | excellent emboss |
| overlapping T | 40 microns | good emboss |

In describing the invention to arrive at a successful product and process the following terms are used:
Emboss: The final pattern introduced during the process on the final polymer layer;
Pattern depth: The depth of the pattern on the Embosser roll;
Emboss depth: The depth of impression between the highest peak and lowest valley of the emboss;
Over-embossing: Embossing that leads to a product with decreased clarity of emboss (due to increased emboss);
Faint emboss: Emboss having a decreased clarity of overall emboss visual effect due to decreased emboss depth;
Dry film thickness: The nominal thickness of the coating layer in microns as produced according to the manufacturing method.

According to the invention the final, outer embossed layer is PVDF.

The coating of a layer of PVDF yields a dry film thickness in the range of 15 - 50 microns. The lower limit is due to inconsistent film formation and the upper limit is due to a defect caused by solvent boil.

It has been found that the product layer structure and composition are important for the overall product performance. Good embossed designs avoiding a product with visual defects can be achieved as long as one works according to one of the following options.

### Option A: Outer polymer layer + primer

The pattern depth should be between 30 and 50 microns. Greater than 50 microns will lead to the emboss pattern exposing the primer and compromising performance. As the coating thickness increases the risk of over embossing increases. For a dry film thickness between 30 microns and 50 microns, a 50 micron pattern depth should be used for a well-defined emboss. For a coating thickness between 15 and 30 microns a lower emboss pattern depth will give a fainter emboss.

### Option B: Outer polymer layer + thermoplastic intermediate + primer

The overall thermoplastic dry film thickness should be 60 microns or smaller in order to avoid over-embossing. The intermediate layer will need to have a certain minimum thickness to achieve the required performance for end use.

For an overall thermoplastic layer dry film thickness between 50 and 60 microns a 50 to 70 micron emboss pattern can be used. An overall thermoplastic coating less than 50 microns can be treated as a single layer as in Option A.

### Option C: Outer polymer layer + thermoset intermediate layer + primer

For an embossed product with an intermediate layer of thermoset chemistry such as PUR. The thickness of the intermediate layer will be the minimum to achieve required performance. The emboss layer should be between 30 and 50 microns. Below this thickness will lead to faint emboss designs. An emboss roll of 50-70 microns can be used.

## Claims

1. Polymer coated sheet product comprising a metallic substrate provided with a polymer coating, the polymer coating comprising an inner polymer layer contacting the metallic substrate and an outer polymer layer wherein an emboss pattern is hot embossed in the outer polymer layer which is of PVDF.

2. Polymer coated sheet product according to claim 1 comprising an intermediate polymer layer extending between the inner polymer layer and the outer polymer layer.

3. Polymer coated sheet product according to claim 1 or claim 2, wherein the inner polymer layer is of polyester, polyurethane or acrylic.

4. Polymer coated sheet product according to claim 1 to 3, wherein the intermediate polymer layer is of polyester, polyurethane or PVDF resin.

5. Polymer coated sheet product according to any of the preceding claims, wherein the dry film thickness of the whole polymer coating is more than 20 microns.

6. Polymer coated sheet product according to any of the preceding claims, wherein the dry film thickness of the whole polymer coating is less than 100 microns.

7. Polymer coated sheet product according to any of the preceding claims, wherein the inner polymer layer has a dry film thickness of 3-30 microns, preferably 5-25 microns.

8. Polymer coated sheet product according to any of the preceding claims, wherein the outer polymer layer has a dry film thickness of 20-70 microns, preferably 30-50 microns.

9. Polymer coated sheet product according to any of the preceding claims 2 to 8 wherein the intermediate polymer layer has a dry film thickness of 10-25 microns.

10. Polymer coated sheet product according to claim 9 wherein the total dry film thickness of the intermediate polymer layer and the outer polymer layer is at least 20 microns.

11. Polymer coated sheet product wherein the metallic substrate comprises a steel sheet.

12. Polymer coated sheet product according to claim 11 wherein the steel sheet has a metallic coating, such as of Zn or a Zn alloy, or a Zn-Mg-Al alloy or of any other metal or alloy.

13. Polymer coated sheet product according to any one of the claims 1 to 10 wherein the metallic substrate comprises an aluminium sheet.

14. Method of manufacturing a polymer coated sheet product having an emboss comprising the following consecutive steps:
- providing a metallic substrate such as S220GD to S550GD or DX51 to DX56 in a suitable gauge ranging from 0.2 to 1.5 mm;
- applying as a first polymer layer an organic primer with a dry film thickness of between 3 and 30 microns, the primer being either polyester or polyurethane or acrylic based and curing the primer;
- optionally applying one or more further polymer layers, the or each further polymer layer being either a colour polymer layer or a base colour polymer layer, having a polyurethane or PVDF chemistry and curing, each colour or base colour polymer layer being preferably between 10 and 30 microns and to be cured preferably between 230 °C and 250 °C;
- applying a final polymer layer being either a clear or a colour PVDF polymer layer with a minimum dry film thickness of 20 microns and a maximum dry film thickness of 70 microns;
- curing the final polymer layer in a curing station preferably at a peak metal temperature of 240 °C to 250 °C;
- embossing the still hot product by passing it through an embosser station as soon as the product exits the curing station whereupon while the product is still hot, a desired pattern is embossed directly into the PVDF final polymer layer, the emboss pattern depth on the embossing roll being preferably 20 microns to 70 microns;
- quenching the final polymer layer by passing the product through a quenching section to cool it whereby the emboss is fixed within the final polymer layer.

15. Method according to claim 14 wherein the metal substrate is coated with a metallic coating on the metal substrate.

16. Method according to claim 15 wherein the metallic coating is a zinc based coating like a Zn coating, a Galvalloy coating, a Galvalume coating, or a Zn-Mg-AI coating, with a coating weight of 60 to 600 grams per square metre.

17. Method according to any of claims 14 to 16 wherein the optionally metallic coated substrate before applying the primer is cleaned involving an alkali cleaning process to remove residual organic matter and metallic oxides.

18. Method according to any of the claims 14 to 17 wherein the optionally metallic coated substrate before applying the primer is pretreated by passing it through a chromate free pretreatment bath based on titanium dioxide or an inorganic component together with an organic polymer to improve the corrosion resistance and enable optimal adhesion between the metallic substrate and subsequent organic polymer layers.

19. Method according to claim 18 wherein the pretreated substrate is rinsed and dried in an oven.
